

April 23, 1946.

J. M. SCHANTZ

2,399,063

LUBRICATING GREASE

Filed March 23, 1944



JACOB M. SCHANTZ  
INVENTOR.

BY *Cleveland B. Hollabaugh*  
ATTORNEY

## UNITED STATES PATENT OFFICE

2,399,063

## LUBRICATING GREASE

Jacob M. Schantz, Wilmington, Del., assignor to  
Hercules Powder Company, Wilmington, Del.,  
a corporation of Delaware

Application March 23, 1944, Serial No. 527,688

14 Claims. (CL 252—37.7)

This invention relates to improved lubricating greases and methods for their production, and more particularly it relates to improved solid lubricating greases containing a hydrogenated rosin soap as an essential ingredient.

It is known in the art that lubricating greases can be prepared by dispersing a metal soap of rosin or rosin oil in a suitable mineral lubricating oil. Generally, a small amount of water is employed in conjunction therewith, the final product being a water-in-oil type emulsion. It has been difficult, however, to prepare solid lubricating greases in this manner without employing large amounts of the metal soap of the rosin or rosin oil. With the employment of large amounts of rosin soap compatibility difficulties are encountered. Either the components are almost entirely incompatible, or they are not sufficiently compatible to yield greases of good uniform texture. Graining and dark colored greases very frequently result. If the metal soap constituent of the grease amounts to as much as 30% or more, black solids result which are entirely useless in practical application. A factor not to be ignored is the fact that the use of such large amounts of metal soap increases the cost of the resulting grease measurably.

Now in accordance with this invention it has been found that these difficulties are largely avoided in a lubricating grease comprising a metal soap of a hydrogenated rosin having at least about 50% of the double bonds contained therein saturated with hydrogen. Such greases are characterized by the marked and unusual gel forming characteristics of the soaps. These greases prepared from soaps of rosin which have been rather highly hydrogenated, have an exceptionally high viscosity which cannot be nearly equalled in greases containing the same amount of metal soaps of rosin known to the prior art. The result is that greases can be prepared in accordance with the processes disclosed herein which contain much less soap than has heretofore been required.

In preparing these new greases it has been found that the above defined hydrogenated rosin may be dissolved in mineral oil, the hydrogenated rosin then saponified by the addition of a desired metal compound with agitation at an elevated temperature, and the remainder of the mineral oil thereafter added. An alternative method involves dissolving a prepared metal salt of the hydrogenated rosin in mineral oil at an elevated temperature and diluting the resulting liquid with additional mineral oil with agitation to achieve the desired concentration of metal soap of the hydrogenated rosin.

In accordance with this invention it is preferred to employ a small amount of water as an

ingredient at some point during the preparation of the grease such that the resulting grease is a water-in-oil type emulsion. It will be understood, however, that the use of water is not absolutely necessary, although desirable. This will be evident from the examples which follow.

Two different procedures were employed in preparing the lubricating greases in the examples. The first procedure involved the preparation of 10 the metal soap, as for example, the calcium soap by saponification in situ. The hydrogenated rosin to be saponified was dissolved in an equal volume of mineral oil and placed in a mixer cup adapted with a stirring mechanism, the cup being immersed in an oil bath. The temperature of the mixture was held at 115° C. and with agitation the addition of a lime-calcium acetate mixture, containing about 5% calcium acetate, was begun together with a few drops of water initially to 15 catalyze the reaction. The remaining portion of the lime was slowly added, care being taken to prevent excessive foaming and loss of sample. After a sufficient amount of the lime-calcium acetate mixture was added to make the theoretical diresinate, the reaction was allowed to continue with agitation at 115° C. When the mixture became plastic and shiny in appearance (apx. 1/2 hr.), heating was discontinued and the remaining portion of the oil slowly added. This final addition of the oil was made slowly at the 20 beginning to minimize the formation of granules and to allow a thorough dispersion. After all the oil was added, the grease was removed from the cup and allowed to set. In those cases where 25 water-in-oil-emulsions were prepared, 1.0% of water on the basis of the finished grease was added with vigorous agitation at 100° C. and the mixture allowed to cool.

The second procedure followed in the examples 30 involved the making of greases from prepared soaps. The desired soap was dissolved in twice its weight of mineral oil by stirring and heating to 175° C., or above if necessary, under an atmosphere of CO<sub>2</sub>. The mixture was then diluted 35 with the required amount of mineral oil, thoroughly agitated and allowed to cool. In the cases of those greases which were water-in-oil emulsions, 1.0% of water was added with agitation at 100° C. and allowed to cool. In all the examples, the mineral oil employed was Sunoco 40 (S. A. E.-20).

A series of greases was made up using prepared 45 soaps made from gum rosin and prepared soaps made from gum rosin which had 69% of the double bonds thereof saturated with hydrogen. These greases were all of the water-in-oil type emulsion, 1.0% water having been added during 50 the preparation. The calcium content of the resinate of I gum rosin and the resinate of 69% hydrogenated I gum rosin was 5.6 and 5.7%, re-

spectively. The resulting greases were tested for consistency on an A. S. T. M. Universal precision penetrometer, the figures given in the following table being the millimeters penetration in 5.0 seconds at 70° F. using a 10.0 gram cone. Other characteristics of the grease were evaluated. The formulations and evaluations follow in Table I. The results are shown graphically in the attached drawing.

Table I

| Calcium soap                   | Percent soap | Consistency | Remarks                            |
|--------------------------------|--------------|-------------|------------------------------------|
| I gum rosin                    | 50.0         | 2           | Black solid.                       |
| Do                             | 40.0         | 40          | Plastic black solid.               |
| Do                             | 30.0         | 280         | Soft black grease of poor texture. |
| Do                             | 20.0         | Liquid      | Incompatible black liquid mixture. |
| 69.0% hydrogenated I gum rosin | 30.0         | 38          | Light transparent solid.           |
| Do                             | 15.0         | 114         | Light colored medium soft grease.  |
| Do                             | 10.0         | 298         | Light colored very soft grease.    |

Referring to the curves on the accompanying drawing, it will be apparent that whereas a satisfactory grease was prepared on the basis of 10% by weight of the calcium soap of the hydrogenated rosin, three times that much, or an increase of 200%, of the calcium soap of I gum rosin had to be employed to make a material of sufficient consistency that it could be called a grease. Even this material was black in color and of poor texture.

It has been found that other hydrogenated rosin soaps may be employed in place of those prepared from 69% hydrogenated rosin. Thus, soaps prepared from hydrogenated rosins having at least about 50% of the double bonds thereof saturated with hydrogen may be employed and they have been found to exhibit this unusually strong gel forming characteristic in conjunction with mineral oils. Tests have shown that soaps prepared from hydrogenated rosins of less than 50% saturation do not exhibit this property to any marked degree.

Another series of greases was made up using direct saponification in situ and substituting a 60% hydrogenated wood rosin in place of the hydrogenated gum rosin employed above. In this series there were included greases made up using mixtures of tallow fatty acids and hydrogenated gum and wood rosins. In all of the greases in this series the finished greases contained 14.6% soap. The greases were all water-in-oil type emulsions, 1.0% water being employed. The saponification time was 60 minutes at a temperature of 115° C. in each case. Where tallow fatty acid was employed as one of the constituents, Emery F-1 fatty acid was used. The formulations and evaluations follow in Table II.

Table II

| Acid constituents                                          | Properties of grease |                           |
|------------------------------------------------------------|----------------------|---------------------------|
|                                                            | Consistency          | Remarks                   |
| (60% hydrogenated wood rosin)                              | 122                  | Transparent grease.       |
| (60% hydrogenated wood rosin) <sup>1</sup>                 | 260                  | Soft, transparent grease. |
| 50% I gum rosin (60% hydrogenated), 50% tallow fatty acid. | 255                  | Soft grease.              |
| 50% wood rosin (60% hydrogenated), 50% tallow fatty acid.  | 235                  | Do.                       |

<sup>1</sup> 10% soap used.

Additional greases were made up on the basis of soaps other than calcium soap. In the preparation of the lead-type grease no water was employed, whereas in the preparation of the barium grease 1% water was employed to form a water-in-oil type emulsion. The lead-type grease was made from a prepared soap containing the theoretical amount of lead for the diresinate, whereas the barium-type grease was made by direct saponification in oil. The properties of the resulting greases are given in the following table in conjunction with those of a grease made from a prepared calcium diresinate of a 60% hydrogenated wood rosin. This particular grease contained 1% water and was a water-in-oil type emulsion. The results follow in Table III.

Table III

| Type grease | Percent soap in grease | Properties of grease |                     |
|-------------|------------------------|----------------------|---------------------|
|             |                        | Consistency          | Remarks             |
| Lead        | 15.0                   | 178                  | Transparent grease. |
| Barium      | 15.0                   | 225                  | Do.                 |
| Calcium     | 20.0                   | 138                  | Do.                 |

The hydrogenated rosin which is utilized in accordance with this invention may be made according to any of the known methods of hydrogenation, as for example, by treatment of the rosin in molten form or in solution in a volatile organic solvent with hydrogen in the presence of a hydrogenation catalyst such as the noble metal catalysts as platinum, rhodium, iridium, ruthenium, palladium, osmium; the base metal catalysts as nickel, nickel-aluminum, nickel-silicon, etc., or the copper chromite type catalysts. The hydrogenation is carried out to provide a hydrogenated rosin in which at least 50% of the double bonds thereof are saturated with hydrogen. Preferably, a hydrogenated rosin having at least 60% of the double bonds thereof saturated with hydrogen will be used.

The rosin employed in the hydrogenation may be wood rosin, gum rosin, or the acids contained therein, as abietic, pimaric, sapinic, etc., acids. Either before or after hydrogenation the rosin may be subjected to vacuum distillation to remove the light end or to remove a particular fraction. If desired, it may be subjected to a refining treatment with a selective color body solvent or adsorbent, as furfural, phenol, fuller's earth, etc.

When, as indicated by the examples, it is desired to prepare a lubricating grease by employing a prepared resinate, the resinate employed may be any of those prepared by methods known to the art. Thus, any of the rosins or modified rosins set forth hereinabove may be hydrogenated by the methods indicated herein and to the extent required in accordance with this invention, and the resulting hydrogenated rosin or modified rosin saponified to form the prepared resinate.

Thus, for example, resinates may be prepared by melting a sample of hydrogenated rosin at an elevated temperature, preferably between about 150° C. and about 316° C. The metal is then added to the melt in the form of the acetate, oxide, hydroxide, or other reactive compound, and the heating is continued until reaction is complete. If desired, the resinates may be prepared by precipitation. Hydrogenated rosin is dissolved in a suitable solvent such as petroleum hydrocarbons, as gasoline, etc., aromatic hydro-

carbons, as toluene, etc., and the desired metal compound added thereto.

Alternatively, any of the aforesaid rosins or modified rosins may be saponified by methods known to the art and the resulting resinates hydrogenated to the degree required in accordance with the invention, i. e., to the point where at least 50% of the double bonds of the rosin or modified rosin are saturated.

It has been found in accordance with this invention that the soaps which have unusually strong gel forming characteristics and which produce particularly satisfactory greases are the calcium, barium and lead soaps; of these, the calcium soap is the most desirable. It will be understood, however, that other mineral oil-soluble soaps of rosin having at least 50% of the double bonds thereof saturated with hydrogen may be employed.

Several of the examples have shown the formation of the soaps of hydrogenated rosin in situ. In preparing greases in accordance with this procedure, the metal compound added may be the acetate, the hydroxide, the oxide or other reactive compound. The negative radical of the compound employed does not have any appreciable effect on the resulting grease. It has been found, however, that the addition of a small amount of water to the mix during the initial reaction will catalyze the reaction. In making greases containing the calcium soap, the use of a calcium oxide-calcium acetate mixture has been found very satisfactory.

In preparing greases by the method wherein the soap is formed in situ, the amount of metal compound employed to saponify the hydrogenated rosin may vary. It is preferred, however, to employ an amount falling within the range between the amount necessary to produce the neutral salt of the acid constituents of the hydrogenated rosin and a 100% excess.

The examples show that the soap concentrations in the improved lubricating greases must be at least about 10.0% by weight. Thus, referring to Table I and the attached drawing, utilizing a calcium soap concentration of 10.0%, the resulting composition was a light colored very soft grease. If soap concentrations below 10.0% by weight are employed, the product is not a solid grease but a liquid not possessing the desired characteristics of a grease.

The lubricating greases prepared in accordance with the invention may contain water emulsified therein to the extent of not more than about 10% based on the weight of the total composition. Generally, a much smaller amount of water will be employed. This water may be added to the grease during preparation or at any time thereafter. The addition should be accompanied by vigorous agitation at a somewhat elevated temperature, as for example, 100° C.

It will be understood that any mineral lubricating oil may be employed in producing these greases, the particular one employed in the examples, i. e., Sunoco (S. A. E.-20), being merely illustrative. Additional lubricating assistants such as graphite, powdered mica, etc., may be added to these greases to the extent of as much as 25% by weight of the composition.

As is illustrated by the examples a fatty acid may be employed in conjunction with hydrogenated rosin in the preparation of desirable greases in accordance with this invention. Thus, for example, tallow fatty acid as Emery F-1 may be employed. When such fatty acids are employed

in conjunction with hydrogenated rosin, satisfactory greases may be obtained using somewhat less than 10% metal soap of hydrogenated rosin on the basis of the finished grease. However, the total amount of metal soap in the greases will be at least 10%.

It will be understood that in preparing these improved greases by the method of saponification in situ the temperature at which the saponification is carried out is not particularly critical. Any temperature may be employed above that at which the particular metal compound employed will react with the hydrogenated rosin. It is important also not to employ a saponification temperature so high that decomposition of the constituents results. As indicated in the examples, the temperature of 115° C. has been found very satisfactory where the metal compound employed is calcium oxide catalyzed with a small amount of calcium acetate. Other optimum temperatures would be employed where different metal compounds are employed for the saponification.

In the preparation of an improved grease in accordance with this invention wherein the grease is made from a prepared soap, the temperature at which the soap-mineral oil mixture is heated is not critical. It is required merely that the temperature be sufficiently high to obtain solution of the soap. The use of an inert atmosphere such as CO<sub>2</sub> during the dissolution process is not absolutely necessary, although desirable.

The improved solid grease prepared in accordance with this invention from hydrogenated rosin having at least about 50% of the double bonds thereof saturated with hydrogen may be variously employed in industry. They are very suitable for chassis lubricants, compression grease cups, gear boxes, and other applications where high speeds and very high temperatures are not encountered. The concentrations of soap in these greases will vary depending upon the desired consistency and specific application.

The advantages of the invention are manifest. The novel greases which are produced in accordance with the herein described processes are characterized by the marked and unusual gel forming characteristics of the soaps. Satisfactory greases can now be compounded employing as little as 10% soap on the basis of the entire composition, whereas heretofore about three times that quantity of soap has been required to produce a solid grease. This involves a considerable conservation of material.

The greases resulting from the improved processes of this invention are of much improved color and texture. Furthermore, the greases are characterized by stability to oxidation. The compatibility difficulties encountered with the heretofore required use of large amounts of rosin soap are largely avoided in the utilization of the greases disclosed herein. At the same time, these greases are not as expensive to manufacture.

This application is a continuation-in-part of my application for U. S. Letters Patent, Ser. No. 412,424, filed September 26, 1941.

Where in the specification and amended claims the term "dissolved" is used in reference to a soap of hydrogenated rosin and mineral oil, there is meant the formation of a homogeneous liquid. Whether this resulting liquid is technically a true solution or a suspension is not known. It is not intended that the application be limited by the terminology employed in this respect.

Where in the specification a particular rosin

is described as "60% hydrogenated," etc., the expression is intended to be equivalent to a rosin having 60% of the double bonds thereof saturated with hydrogen.

What I claim and desire to protect by Letters Patent is:

1. A lubricating grease comprising a mineral oil-soluble soap of a rosin having at least about 50% of the double bonds thereof saturated with hydrogen, in conjunction with a mineral oil, said soap being present in the amount of at least about 10.0% by weight of the finished grease.

2. A lubricating grease comprising a mineral oil-soluble metal soap of a rosin having at least about 50% of the double bonds thereof saturated with hydrogen, in conjunction with a mineral oil, said metal being selected from the group consisting of calcium, barium, and lead, said soap being present in the amount of at least about 10.0% by weight of the finished grease.

3. A lubricating grease comprising the calcium soap of a rosin having at least about 50% of the double bonds thereof saturated with hydrogen, in conjunction with a mineral oil, said soap being present in the amount of at least about 10.0% by weight of the finished grease.

4. A lubricating grease comprising the barium soap of a rosin having at least about 50% of the double bonds thereof saturated with hydrogen, in conjunction with a mineral oil, said soap being present in the amount of at least about 10.0% by weight of the finished grease.

5. A lubricating grease comprising the lead soap of a rosin having a least about 50% of the double bonds thereof saturated with hydrogen, in conjunction with a mineral oil, said soap being present in the amount of at least about 10.0% by weight of the finished grease.

6. A lubricating grease comprising a mineral oil-soluble soap of a rosin having at least about 60% of the double bonds thereof saturated with hydrogen, in conjunction with a mineral oil, said soap being present in the amount of at least about 10.0% by weight of the finished grease.

7. A lubricating grease comprising a mineral oil-soluble soap of a rosin having at least about 60% of the double bonds thereof saturated with hydrogen, in conjunction with a mineral oil and a small amount of water, said soap being present in the amount of at least about 10.0% by weight of the finished grease.

8. A lubricating grease comprising a mineral oil-soluble soap of a rosin having at least about 60% of the double bonds thereof saturated with hydrogen, in conjunction with a mineral oil and not more than 10% water on the basis of the finished grease, said soap being present in the amount of at least about 10.0% by weight of the finished grease.

9. A lubricating grease comprising the calcium soap of a rosin having at least about 60% of the double bonds thereof saturated with hydrogen, in conjunction with a mineral oil, said soap being present in the amount of at least about 10.0% by weight of the finished grease.

10. A lubricating grease comprising the barium soap of a rosin having at least about 60% of the double bonds thereof saturated with hydrogen, in conjunction with a mineral oil, said soap being present in the amount of at least about 10.0% by weight of the finished grease.

11. A lubricating grease comprising the lead soap of a rosin having at least about 60% of the double bonds thereof saturated with hydrogen, in conjunction with a mineral oil, said soap being present in the amount of at least about 10.0% by weight of the finished grease.

12. A lubricating grease comprising a mineral oil-soluble soap of a rosin having at least about 50% of the double bonds thereof saturated with hydrogen and a mineral oil-soluble soap of a fatty acid, in conjunction with a mineral oil, said soap of a rosin being present in the amount of at least about 10.0% by weight of the finished grease.

13. A lubricating grease comprising the calcium soap of a rosin having at least about 60% of the double bonds thereof saturated with hydrogen, in conjunction with a mineral oil and a small amount of water, said soap being present in the amount of at least about 10.0% by weight of the finished grease.

14. A lubricating grease comprising the barium soap of a rosin having at least about 60% of the double bonds thereof saturated with hydrogen, in conjunction with a mineral oil and a small amount of water, said soap being present in the amount of at least about 10.0% by weight of the finished grease.

JACOB M. SCHANTZ.